

## UNITED STATES PATENT OFFICE

2,226,284

## METHOD FOR PREVENTING INTERGRANULAR OXIDATION IN TERNARY BERYLLIUM ALLOYS

Richards H. Harrington, Schenectady, N. Y., assignor to General Electric Company, a corporation of New York

No Drawing. Application July 29, 1938,  
Serial No. 221,976

1 Claim. (Cl. 148—13.2)

The present invention relates to ternary alloys containing copper, beryllium and metal from the group cobalt and chromium but more particularly to a method for producing such alloys in the form of wire or strip. Alloys of this composition are disclosed in Dahl Patent 1,847,929 and in Horstkotte Patent 1,957,214 and heretofore have been employed to a considerable extent as forged material and castings and in the form of welding electrodes and current conducting bearings. In fabricating the alloys a heat treatment is employed to effect precipitation hardening. This treatment consists in heating the alloys to a temperature of about 900° C. to effect a solid solution condition in the alloy, quenching and thereafter reheating or drawing the alloy at 450° C. to 550° C. to effect a condition of precipitation in the alloy.

In heating these alloys at temperatures above 500° C. a certain amount of intergranular oxidation takes place. Such oxidation generally is not detrimental in castings, rod or plate stock since they usually are not subjected to permanent bending and when that is necessary they may be machined before bending to thereby remove the oxidized surface. The intergranular oxidation condition however is particularly undesirable when these alloys are in the form of strip or wire since the latter owing to their small cross sectional area are particularly sensitive to intergranular oxidation. When such a condition exists in the wire or strip alloys they crack severely when bent thereby rendering the material useless for purposes such as springs and the like.

One of the objects of the present invention is to provide means for preventing intergranular oxidation in alloys, in strip or wire form, which consist of copper, cobalt and beryllium or copper, chromium and beryllium.

In carrying out the present invention, the alloys are heated as heretofore at a temperature about 900° C. and for a period of time sufficient to effect a solid solution condition in the alloys but the heating, contrary to the former practice, is carried out in a protective atmosphere free from oxygen, carbon dioxide and water vapor. The alloy strip or wire is then quenched from the solution temperature. The quenching medium may be oil but more satisfactory results are obtained by quenching in a 10% salt water solution.

If any appreciable quantity of oxygen, carbon dioxide or water vapor is present in the furnace atmosphere, intergranular oxidation of the alloy wire or strip will take place. Partially combusted city gas, cracked ammonia, or substantially any gaseous medium from which oxygen, carbon dioxide and water vapor have been removed may be employed as the furnace atmosphere. When the strip or wire which has been heated in the controlled atmosphere is quenched in oil the freedom from intergranular oxidation is maintained. However, the physical properties of the alloy quenched in oil are inferior to the properties obtained with a salt water quench. If the alloy is quenched in water to which salt has been added the salt solution acts to break up any vapor film which otherwise might form on the surface of the hot metal when it is plunged into the cooling medium and thereby prevents any intergranular oxidation during quenching. After quenching from the solution temperature the alloy wire or strip may be precipitation hardened by reheating or drawing at the usual elevated temperatures but not materially higher than 500° C. and for the usual periods of time necessary to effect the condition of precipitation in the alloys. If the draw or reheat is carried out in air the alloy strip or wire should be pickled thereafter to remove any scale formed during the draw or reheat. The alloys may be cooled from the reheat temperature in air or in gaseous atmospheres which ordinarily prevent scaling at 500° C. Any scale which may be formed during the draw is not accompanied by intergranular oxidation, since the latter occurs only at temperatures above 500° C.

What I claim as new and desire to secure by Letters Patent of the United States is:

The method of preventing intergranular oxidation in wire or strip ternary alloys consisting of copper, beryllium and metal from the group cobalt and chromium which comprises heating said alloys to an elevated temperature in an atmosphere free from oxygen, water vapor and carbon dioxide to thereby effect a solid solution condition in the alloy and quenching said strip or wire from said temperature in a salt solution.

RICHARDS H. HARRINGTON.

50